

## UNITED STATES PATENT OFFICE

2,255,895

## WORKABLE NICKEL AND NICKEL ALLOY

Leonard Bessemer Pfeil, Edgbaston, Birmingham, England, assignor to The International Nickel Company, Inc., New York, N. Y., a corporation of Delaware

No Drawing. Original application October 6, 1936, Serial No. 104,179. Divided and this application April 25, 1939, Serial No. 269,912. In Great Britain October 15, 1935

6 Claims. (Cl. 75—171)

The present invention relates to nickel and nickel alloys having improved workability and products made therefrom including electric resistance units.

Nickel and its alloys have, in some cases, been somewhat difficult to work and under certain circumstances an alkaline earth metal has often been added to the molten materials. In order to obtain the full benefits of the addition of the alkaline earth, it is desirable to add more of the alkaline earth metal, calcium for example, than is consumed by the desired chemical reactions. This results in a residue of calcium or other alkaline earth in the finished material (or a residue of some other element reduced from the furnace lining, slag, and so forth, by the excess calcium, etc.), but it is important to control the amount of alkaline earth metal that is left as the presence of more than a certain amount of calcium or other alkaline earth metal makes the material unworkable.

I have made the surprising discovery that the necessity for strict control of the amount of calcium or other alkaline earth metal can be avoided and yet the materials can be rendered easily workable.

It is an object of the present invention to provide nickel and/or nickel alloys having improved workability.

It is another object of the present invention to provide means for obviating the need for extreme care in regulating the amount of alkaline earth metal added to nickel and/or nickel alloys.

It is a further object of the present invention to compensate for the excess of alkaline earth present in a nickel and/or nickel alloy material by the addition of a regulated, critical amount of another element usually considered deleterious.

The present invention also contemplates the production of nickel alloys particularly suitable for use as electrical resistance units.

Other objects and advantages will become apparent from the following description.

In general, the present invention contemplates melting nickel and/or nickel alloying metals in the usual manner followed by the usual deoxidizing, desulfurizing, etc. The deoxidizing, desulfurizing, etc., may be carried out by the addition of calcium silicide or other alkaline earth metals or alkaline earth metal alloys, or by means of aluminum, cerium and related elements (including thorium, hafnium, scandium, yttrium, and zirconium); and man-

ganese, molybdenum, silicon and titanium may be added with advantage. Other elements that may be added are barium, beryllium, boron, cobalt, copper, lithium, magnesium, strontium, sulfur, and tungsten. Moreover, more than one of the alkaline earth metals may be added to the melt, whether or not more than one such metal is left in the finished material, and similarly more than one of the metals usually considered deleterious may be added.

It is convenient to describe the nature of the present invention in connection with calcium and arsenic, but it is to be understood that these may be replaced respectively by other alkaline earth metals and other elements of group V, i. e., phosphorus, antimony and bismuth.

The amount of calcium and the accompanying arsenic to be added to the melt varies according to the working conditions, i. e., the type of furnace, conditions of the lining, the speed of melting, the nature of the raw materials, and other similar factors, but in order to give an indication of the relative amounts of calcium and arsenic, it may be stated that when between 25 about 0.05 and about 0.15% calcium is present in the finished material that may advantageously be accompanied by about 0.01 to about 0.05% arsenic. In general, it is preferred so to carry on the process that small quantities of 30 calcium and an element of group V remain in the finished material because in this way, it can be ensured that the beneficial effects obtained by their addition to the molten material are produced to the full. The preferred ranges 35 are as follows:

| Element: | Per cent<br>by weight | Element:    | Per cent<br>by weight |
|----------|-----------------------|-------------|-----------------------|
| Calcium— | 0.01 to 0.10          | Phosphorus— | 0.01 to 0.06          |
| Calcium— | 0.01 to 0.15          | Arsenic—    | 0.01 to 0.2           |
| Calcium— | 0.01 to 0.2           | Antimony—   | 0.01 to 0.25          |

40 In the case of bismuth, not more than about 0.075% should be added.

As is well known, the calcium may be added as a metal or as an alloy or compound, such as calcium silicide and the group V element may 45 be added in the elemental form or as an alloy or compound, such as, for example, nickel arsenide or calcium phosphide. The alloying process may be carried out in any suitable manner. Thus, a preliminary addition of calcium silicide may be made to the melt and any substantial excess of calcium removed by oxidation. A final calcium silicide addition may be made just before casting. The less oxidizable of the group V elements may be added at any stage in the melt-

ing process, or may be added in a suitable alloyed form with the cold charge.

The additions may be made by plunging the elements or alloys to the bottom of the molten metal by any suitable means so as to improve the alloying process. The group V elements together with part or all the calcium, or other alkaline earth metal, may, however, be added to the molten stream during the pouring of the metal.

For the purpose of giving those skilled in the art a better understanding of the present invention, the following examples are given by way of illustration.

#### Example No. 1

In the production of the well known 80/20 nickel-chromium alloy according to the present invention, the following procedure may, for example, be followed:

About 800 pounds of nickel are melted and subjected to deoxidation by the addition of about 0.25 to about 0.5% manganese and about 0.25% silicon, about 200 pounds of chromium are added and when the mass is molten, about 6 pounds of calcium silicide containing about 25% calcium are added. This is equivalent to adding about 0.13% calcium to the melt. When sufficient time has been allowed for the desired reactions to proceed and the temperature of the metal has been adjusted to that correct for casting, the metal is poured into a ladle, and about 0.5 of a pound of metallic arsenic is added thereto. About 1 pound of calcium silicide is introduced into the ladle, and the metal is cast. These last additions represent about 0.045% and about 0.08%, respectively, of the total mass.

#### Example No. 2

The procedure of Example No. 1 is followed until the chromium has been added to the melt, and then about 4 pounds of the calcium silicide and, for example, about 1 pound of commercial cerium are added. The melt is poured into the ladle while adding about 0.25 pound of metallic arsenic. About 0.50 pound of calcium silicide and about 1 pound of cerium are added while the metal is in the ladle.

#### Example No. 3

As illustrative of the process according to the present invention as applied to the production of nickel, the following example is given:

About 1000 pounds of commercial nickel are melted together with about 0.25% manganese and about 0.1% silicon. When molten, the metal is poured into the ladle and during the pouring operation, an addition of about 0.025% arsenic is made followed by about 0.05% calcium either in the metallic form or in the form of calcium silicide.

In the application of the present invention to the preparation of iron-nickel alloys, the following example is presented for illustrative purposes:

#### Example No. 4

In the production of 50-50 nickel-iron alloy, about 500 pounds of nickel and about 500 pounds of iron are melted together with about 0.25% manganese and about 0.1% silicon. When molten, the metal is poured into the ladle and during the pouring operation an addition of about 0.025% arsenic is made followed by the addition of about 0.05% calcium either in the metallic form or in the form of calcium silicide.

The present invention may be applied with

particular advantage to those nickel-chromium and nickel-chromium-iron alloys from which, as a general rule, electrical resistance elements are made. As those skilled in the art know, such electrical resistance alloys are also known as high temperature resistance alloys, high resistance alloys, and the like, and include such alloys as are available for use at elevated temperatures in excess of 500° C. Those skilled in the art have classified the nickel-containing alloys in two groups. For instance, Hunter and Jones in an article entitled "Some electrical properties of high-resistance alloys," in the Proceedings of the American Society for Testing Materials, volume 24, 1924, part II, page 401, referred to both the nickel-chromium alloys and the nickel-chromium-iron alloys. Hunter and Jones stated that binary nickel-chromium alloys containing up to 30% chromium had been made and that the commercial alloys usually contained 15% to 20% chromium. The authors also stated that a well known nickel-chromium-iron alloy contained about 60% nickel, 26% iron, and 12% chromium, while another contained less iron and more chromium. It was also pointed out that many of the alloys were worked under the Marsh patent. The Marsh United States Patent No. 811,859 of 1906 disclosed the use of nickel-chromium alloys for electric resistance elements. Marsh's alloys contained over 50% nickel or cobalt, or both, and less than 50% chromium, but preferably contained less than 25% chromium and more than 75% nickel. As examples, the 90/10 and 85/15 nickel-chromium alloys were cited. It was later determined that the best alloy of the series was the 80/20 nickel-chromium alloy. Liddell's Handbook of Non-Ferrous Metallurgy, McGraw-Hill, 1926, volume 2, page 1315, referred to the nickel-chromium and nickel-chromium-iron alloys for heating elements and stated that the commercial alloys contain 5% to 20% chromium, 5% to 40% iron and the balance nickel. The Dempster United States Patent No. 901,428 of 1908 had disclosed the use of nickel-chromium-iron alloys for electric resistance elements. The Dempster alloys contained more than 10% and less than 50% iron, for example, 20% iron. A typical alloy was composed of 62% nickel, 20% iron, 12.6% chromium and about 5% manganese. "The Book of Stainless Steels" edited by Thum and published by the American Society for Steel Treating, 1933, first edition, page 426, contained a section devoted to "Electric resistors" by Hunter, in which typical compositions of some commercial alloys were given. The two outstanding alloys were stated to be the nickel-chromium alloy containing 80% nickel and 20% chromium and the nickel-chromium-iron alloy containing 60% nickel, 25% iron and 12 to 15% chromium. Hunter stated that it was commercially practicable to make binary nickel-chromium alloys containing up to 30% chromium. Hunter stated that the alloys may contain carbon, manganese, silicon, aluminum, molybdenum, copper, etc., in small amounts, for example, 0.07% or 0.1% up to over 2%, and in some instances, for example, molybdenum, as high as 10%. Briefly stated, the nickel-containing alloys adapted for use as electrical heating elements usually contain about 10% to about 30% chromium or more and the balance nickel or nickel and iron with or without some cobalt, the nickel content of the alloys generally exceeding about 50% nickel, i. e., the balance is metal of the iron group of which at least 50% of the alloy is preferably nickel. From their

nature, these alloys give rise to substantial difficulty during the wire producing processes on which the life of the wire may depend. Accordingly, the invention includes electrical resistance elements made from such alloys embracing small quantities of one or more alkaline earth metals and one or more of the group V elements, i. e., phosphorus, arsenic, antimony, etc.

The present application is a division of my co-pending patent application Serial No. 104,179, filed October 6, 1936, which, subsequent to the filing of this application, matured into U. S. Patent No. 2,159,048.

While the present invention has been described in connection with certain preferred embodiments, it is to be understood that variations and modifications may be made by those skilled in the art. Such variations and modifications are considered to be within the spirit and scope of the appended claims.

It is to be understood that the term deoxidation, as used herein, includes such preliminary treatment as deoxidizing, desulfurizing, etc.

I claim:

1. As an article of manufacture, an electrical resistance element made of an improved workable nickel alloy comprising about 10% to about 30% chromium, about 0.01% to about 0.2% calcium, about 0.01% to about 0.25% of at least one of the elements of the group consisting of phosphorus, arsenic and antimony, and the balance substantially all nickel.

2. A nickel alloy possessing improved workability comprising about 10% to about 30% chromium, about 0.01% to about 0.2% calcium, about 0.01% to about 0.25% of at least one of the elements of the group consisting of phosphorus, ar-

senic and antimony, and the balance substantially all nickel.

3. As an article of manufacture, an electrical resistance element made of an improved workable nickel alloy comprising about 10% to about 30% chromium, about 5% to about 40% iron, about 0.01% to about 0.2% calcium, about 0.01% to about 0.25% of at least one of the elements of the group consisting of phosphorus, arsenic and antimony, and the balance substantially all nickel.

4. A nickel alloy possessing improved workability comprising about 10% to about 30% chromium, about 5% to about 40% iron, about 0.01% to about 0.2% calcium, about 0.01% to about 0.25% of at least one of the elements of the group consisting of phosphorus, arsenic and antimony, and the balance substantially all nickel.

5. A nickel-base alloy adapted for use as an electrical heating element comprising about 10% to about 30% chromium, about 0.01% to about 0.2% alkaline earth metal, and at least one of the elements of the group consisting of phosphorus, arsenic and antimony within the range of about 0.01% to about 0.06%, about 0.01% to about 0.2%, and about 0.01% to about 0.25%, respectively, and characterized by high workability compared to a similar alloy free from phosphorus, arsenic or antimony.

6. A nickel-base alloy containing from about 0.01% to about 0.2% of alkaline earth metal, about 0.01% to about 0.25% of at least one element from the group consisting of phosphorus, arsenic and antimony, and characterized by high workability compared to a similar alloy free from phosphorus, arsenic or antimony.

LEONARD BESSEMER PFEIL,